

## UNITED STATES PATENT OFFICE

WILLIAM H. SEAMAN, OF HAMMOND, INDIANA

## METAL ROLL

No Drawing.

Application filed June 27, 1927. Serial No. 201,968.

My invention relates to metal rolls for rolling metal articles such as metal strips, sheets and all manner of shapes, and particularly to rolls of this kind known as chilled iron alloy rolls because of their being cast in a chilled mold or in a sand mold with sufficiently heavy condensing chills.

The principal object of the invention is to provide a roll of the class specified which shall have certain highly desirable characteristics or qualities such as toughness, durability, hardness, freedom from fire cracking, and shall also have a particularly hard outer portion especially advantageous for rolling and advantageously associated with the remainder of the roll.

The roll herein set forth for carrying out the invention, is a chilled cast iron alloy roll having a substantial or high carbon content running usually from about 3% to 3.75% and also having certain other modifying ingredients, such as manganese, silicon, sulphur, phosphorus, chromium and nickel, although not necessarily all of these ingredients or elements. The manganese will run from about .35% to .50%; the sulphur from approximately .05% to .15%; the phosphorus from about .10% to .40%; the silicon from about .75% up, preferably to from .90% to 1.50%; the chromium from about .45% up, preferably running from about .75% to 2.00%; the nickel when used will be preferably in excess of .20% and running from that amount up to 1.00% or even more. Some variation is permissible in all these elements or ingredients. Enough iron is used in addition to the foregoing to make up the total of 100%.

The silicon and chromium, it will be noticed, are in substantial amounts and give the roll certain desirable qualities or characteristics. When the roll is cast either in a chill mold or in a sand mold with sufficiently heavy condensing chills, an outer or primary chill is formed on the outside of the roll and also an inner or secondary chill just inside of the primary chill. The primary chill is a hard skin or layer of solid close grained white iron and the secondary chill

primary chill. Gray or mottled iron forms the central portion of the roll. The secondary chill has no clear line of demarkation between itself and the primary chill and the gray iron center or core. In a roll of substantially the constituency above set forth, the primary chill will be quite thin or small and, on the other hand, the secondary chill will be of very substantial thickness or size. In one type of roll, for example, the primary chill will be perhaps an eighth or quarter of an inch in thickness and the secondary chill from one to two inches thick. This produces a very advantageous form of roll because the primary chill is very tough and hard and not likely to break or crack or separate from the roll and the secondary chill forms a very effective cushion for the primary chill and an effective connection between the primary chill and roll center or core and also a very good structure for rolling shapes.

These chills, the primary and secondary, may be varied in absolute and relative size by variation in the amount of silicon and chromium. The depth or size of the primary chill is controlled quite largely by the amount of silicon used, the size or thickness of the chill being less as the amount of silicon increases, and vice versa. Similarly, the depth or thickness of the secondary chill is largely controlled by the amount of chromium used, this secondary chill being greater as the amount of chromium increases and less as the amount of chromium decreases.

It will be understood that changes and modifications may be made without departing from the spirit of the invention.

What I claim is:

1. A high carbon chilled iron alloy roll having small quantities of modifying elements including an appreciable quantity of nickel and also having substantial quantities of hardening and toughening elements and having a close grained white iron primary chill and a secondary chill having no distinct line of demarkation between it and the primary chill and having a grain structure resembling that of the primary chill.

2. A high carbon chilled iron alloy roll having small quantities of manganese, sul-

phur and phosphorus in excess of .10% and also having substantial quantities of chromium and silicon and having a close grained white iron primary chill and a secondary chill having no distinct line of demarkation between it and the primary chill and having a grain structure resembling that of the primary chill.

3. A high carbon chilled iron alloy roll having small quantities of manganese, sulphur, phosphorus and an appreciable quantity of nickel and also having substantial quantities of chromium and silicon and having a close grained white iron primary chill and a secondary chill having no distinct line of demarkation between it and the primary chill and having a grain structure resembling that of the primary chill.

4. A high carbon chilled iron alloy roll having small quantities of manganese, sulphur, phosphorus in excess of .10% and nickel and also having silicon and chromium each in amount between 1% and 2% and having a close grained white iron primary chill and a secondary chill having no distinct line of demarkation between it and the primary chill.

5. A high carbon chilled iron alloy roll having from 3.00% to 3.75% carbon, about .35% to .50% manganese, about .05% to .08% sulphur, about .20% to 1.00% nickel and from about 1.00% to 1.50% silicon and about .75% to 2.00% chromium and having a close grained white iron primary chill and a secondary chill having no distinct line of demarkation between it and the primary chill and having a grain structure resembling that of the primary chill and a gray or mottled iron core underlying the secondary chill.

6. A chilled cast iron roll containing total carbon about 3.00% to 3.75%, chromium about .70% to 1.25%, phosphorous from about .10% to about .40%, sulphur not over about .10%, silicon about .50% to 1.50%, and manganese about .35% to .50% and having a close grained white iron primary chill and a secondary chill having no distinct line of demarkation between it and the primary chill and having a grain structure resembling that of the primary chill, and a gray or mottled iron core underlying the secondary chill.

In witness whereof, I hereunto subscribe my name this 24th day of June, A. D., 1927.

WILLIAM H. SEAMAN.